

# United States Patent

Robertshaw et al.

[15] 3,640,704

[45] Feb. 8, 1972

[54] **HIGH-TEMPERATURE-STRENGTH,  
PRECIPITATION-HARDENABLE,  
AUSTENITIC, IRON-BASE ALLOYS**

[72] Inventors: **Fred C. Robertshaw, Cincinnati; Jon L. Bartos, Loveland; James J. Hurst, Clarksville; James August McGurty, Cincinnati, all of Ohio**

[73] Assignee: **The United States of America as represented by the United States Atomic Energy Commission**

[22] Filed: **Jan. 20, 1970**

[21] Appl. No.: **4,374**

[52] U.S. Cl. .... **75/128 W, 75/128 R**

[51] Int. Cl. .... **C22c 39/20**

[58] Field of Search ..... **75/128**

[56] **References Cited**  
**UNITED STATES PATENTS**

|           |         |               |          |
|-----------|---------|---------------|----------|
| 2,725,493 | 11/1955 | Mitchel ..... | 75/128 R |
| 3,362,855 | 1/1968  | Shimo .....   | 75/128 R |
| 3,547,625 | 12/1970 | Bieber .....  | 75/128 R |

*Primary Examiner*—Hyland Bizot  
*Attorney*—Roland A. Anderson

[57] **ABSTRACT**

This invention is for an iron-base alloy system characterized in that (a) it consists of an iron-nickel-chromium matrix which maintains substantially complete austenitic stability at temperatures from room temperature to the melting point; (b) it is susceptible to treatment to effect a precipitation-hardening resulting in a molybdenum-containing precipitated phase; (c) said alloy consists essentially of, in atom percent, 20 to 30 percent nickel, 5 to 10 percent chromium, a strength-inducing additive selected from either molybdenum or tungsten in an amount not exceeding 10 percent, and the balance iron.

**3 Claims, 2 Drawing Figures**



FIG. 1

## INVENTORS.

Fred C. Robertshaw  
James A. McGurty  
James J. Hurst  
Jon L. Bartos

BY *Fred C. Robertshaw*

ATTORNEY.



Fig. 2

INVENTORS.  
 Fred C. Robertshaw  
 James A. McGury  
 James J. Hurst  
 Jon L. Bartos  
 BY *Ronald G. Grubbs*  
 ATTORNEY.

## HIGH-TEMPERATURE-STRENGTH, PRECIPITATION-HARDENABLE, AUSTENITIC, IRON-BASE ALLOYS

### BACKGROUND OF THE INVENTION

The invention described herein was made in the course of, or under, a contract with the U.S. Atomic Energy Commission.

The present invention relates to a selected class of precipitation-hardenable iron-base alloys containing nickel, chromium, molybdenum, and tungsten in specifically defined ranges of concentration to ensure a stabilized austenitic (i.e., face-centered cubic or gamma) crystallographic phase over the full range of temperature from 0° C. up to the melting point. While the iron-base alloys of this invention are not steels, they do contain carbon in extremely low quantities, in the parts-per-million range, which do not critically determine any phase relationship or physical property of the herein-described alloy system.

It is a general object of this invention to provide an iron-nickel-chromium-molybdenum or tungsten-containing alloy system capable of being hardened by a precipitation heat treatment to achieve a practical combination of hardness, ductility, short-term and long-term (creep) strength under sustained operation at low and particularly at high (550°-750° C.) service temperatures. A specific object is to provide a stabilized iron-base face-centered cubic alloy system with a creep strength at a temperature in the range 550° to 750° C. which is at least equal to or superior to austenitic stainless steels having useful properties in the same range of temperature.

### SUMMARY OF THE INVENTION

The inventive concept herein disclosed is based on a process of judicious selection of alloy components which enable the definition of an alloy system characterized by a stabilized austenitic crystallography over the temperature range 0° to 1,400° C. This means that the maximum physical properties of the alloy can be utilized without experiencing the changes or discontinuities normally accompanying crystallographic phase transformations in iron-base alloy systems. In addition, the alloy system is precipitation-hardenable to a microstructure which is stable over long periods of time at elevated temperatures without overaging to a brittle condition. The alloy is easily fabricable by standard forming techniques into a variety of forms and shapes; for example, into sheet or tube form. Such an alloy system, in accordance with our invention, consists essentially of, in atom percent, 20-30 percent nickel, 5-10 percent chromium, 5-10 percent of a strength-inducing element selected from the group molybdenum or tungsten, and the balance iron. The phrase "consisting essentially of" is used in this specification to denote positive recitation of essential alloying ingredients but is not meant to rule out the presence of residual amounts of such elements as, by way of example, carbon, boron, and oxygen which are not deliberately added to the alloy for any specific alloying purpose but which occur in low concentrations of the order of from less than 5 to no more than 100 parts per million as impurities which accompany the alloy fabrication process.

The principal criteria for selecting the alloy compositional limits are based on the multifold object of arriving at stable crystallography and microstructure over a wide range of temperature and particularly over the temperature range 550°-750° C. with satisfactorily high short-term and long-term (creep) properties in a nonoxidizing and/or corrosive atmosphere such as liquid sodium where a satisfactory level is measured against the properties of Type 316 stainless steel (16-18 weight percent chromium, 10-14 weight percent nickel, 2-3 weight percent molybdenum, 1 (max.) weight percent silicon, 0.03-0.08 weight percent carbon, plus phosphorus and sulfur).

At the chromium and molybdenum levels of interest here, maximum austenite stability is achieved at nickel concentrations in the range 20-30 percent. Satisfactorily high short-term and long-term strength is attained throughout this nickel range but, where the alloy is exposed to liquid sodium, op-

timum sodium corrosion resistance is obtained with nickel concentrations in the range 20-25 percent.

Molybdenum or tungsten is used in the alloy at concentrations which exceed its room temperature solubility, requiring a minimum of about 4 percent of either metal. The presence of molybdenum or tungsten at these concentrations permits attainment of a uniform precipitation-hardenable dispersed phase within an iron-nickel-chromium matrix produced by suitable solid solutioning followed by subsequent heat treatment at a lower temperature at least equal to or greater than the intended service temperature to develop and sustain a maximum hardness while avoiding the formation of brittle phases. Concentrations of molybdenum, tungsten alone, or the combination of both which exceed 10 atom percent of the total alloy are undesirable because of degradation of ductility due to the formation of a brittle sigma phase.

The presence of chromium in the range of 5 to 10 percent at the prescribed nickel level with a molybdenum and/or tungsten concentration in the range of about 5 to 10 percent has been found to enhance the stability of the austenite phase. In addition, the combination of chromium and the strength-inducing additive appears to enhance high-temperature strength, especially at temperatures in the range 550°-750° C.

Furthermore, the essential absence of carbon avoids the common problem experienced with austenitic chromium-nickel-containing steels of intergranular corrosion due to the formation of precipitated chromium carbides which rob the grain boundaries of the protective effect of chromium.

The phase stability effect of chromium becomes less apparent at concentrations less than 5 percent unless greater amounts of nickel are used within the nickel limits previously described. Thus we have found that a ternary iron-base alloy containing 20 percent nickel, 5 percent molybdenum, and no chromium is unstable and transforms to the body-centered cubic phase, whereas increasing amounts of chromium stabilize the face-centered cubic condition and a 5-percent-chromium addition guarantees stability.

The alloys falling within the scope of this invention are easily fabricable by standard metallurgical techniques such as casting or powder metallurgy. We have found that large pure castings are easily made by vacuum induction melting using a zirconia or alumina crucible. For example, in excess of 3-kilogram vacuum-induction-melted castings have been produced which uniformly contain less than about 15 parts per million carbon, less than 10 parts per million nitrogen, and less than 200 parts per million oxygen, as well as less than 5 parts per million boron, with trace amounts of residual elements such as silicon, sulfur, and titanium, the exact amount depending, apparently, upon the composition of the crucible. In any event, the resultant ingot can be extruded at a temperature ranging from 1,100° to 1,200° C. to an approximately 2-centimeter-diameter rod which can be subsequently forged at the same temperature range to a lesser thickness and then rolled at 1,150° C. to a 0.254-centimeter-thick sheet which can be subsequently cold-rolled or hot-rolled to 0.5-centimeter-thick sheet. Cold-rolling to the required thickness is facilitated by several immediate anneals at temperature of 1,000° to 1,250° C.

The following description provides a representative embodiment of the invention, given in terms of experimental data which illustrate characteristic features of the claimed alloy system of phase stability and high-temperature physical properties as well as illustrating the advantages achieved by precipitation-hardening in improving high-temperature physical properties. The data given in the description are for a preferred alloy of the claimed alloy system which contains 20 percent nickel, 5 percent chromium, and 10 percent molybdenum and represent an excellent combination of phase stability, uniform microstructure, and high-temperature short-term tensile as well as high-temperature (creep) properties.

#### Phase Stability

A vacuum induction melt made from an alloy consisting of 75 20 percent nickel, 5 percent chromium, 10 percent molyb-

denum, and the balance iron was extruded and swaged at 982° C. and subsequently drawn to a test specimen cylinder 0.635 centimeter in diameter by 3.82 centimeters long. Linear thermal expansion coefficients at several temperatures from 0° to 1,400° C. were measured and the results are shown in Table I.

necessary to produce a maximum hardening at aging temperatures from 550° to 850° C. It should, however, be recognized that other combinations of heat treatment may also produce a desirable optimum hardness resulting from precipitation-inducing heat treatments.

TABLE II.—EFFECT OF HEAT TREATMENT ON THE TENSILE PROPERTIES <sup>a</sup> OF  
Fe-20Ni-5Cr-10Mo

| Alloy heat No.             | Condition                                             | Test temp., °C.   | Yield strength <sup>a</sup> |                      | Tensile strength |                      | Elongation, percent |
|----------------------------|-------------------------------------------------------|-------------------|-----------------------------|----------------------|------------------|----------------------|---------------------|
|                            |                                                       |                   | K.s.i.                      | kg./cm. <sup>2</sup> | K.s.i.           | Kg./cm. <sup>2</sup> |                     |
| MS-70 <sup>b</sup>         | Sol. 1,205° C./1 hr. water quenched, then aged        | R.T.              | 64.6                        | 4,520                | 140.6            | 9,900                | 3.6                 |
|                            |                                                       | 550               | 52.1                        | 3,650                | 111.1            | 7,880                | 8.2                 |
|                            |                                                       | 750° C.-50 hours. | 650                         | 44.4                 | 3,100            | 82.9                 | 27.9                |
|                            |                                                       | 750               | 37.6                        | 2,640                | 50.6             | 3,540                | 45.9                |
| MS-70                      | Finished-rolled at 1,150° C. and aged 750° C.-50 hrs. | R.T.              | 63.7                        | 4,450                | 113.3            | 7,930                | 18.5                |
|                            |                                                       | 550               | 53.1                        | 3,730                | 88.2             | 6,200                | 15.7                |
|                            |                                                       | 650               | 47.3                        | 3,310                | 68.7             | 4,800                | 39.4                |
|                            |                                                       | 750               | 37.9                        | 2,650                | 47.9             | 3,350                | 46.6                |
| Type d. <sup>c</sup> 316SS | Annealed 1,120° C.-20 min.                            | R.T.              | 35.7                        | 2,500                | 83.2             | 5,820                | 72.5                |
|                            |                                                       | 550               | 16.0                        | 1,120                | 64.0             | 4,580                | 42.5                |
|                            |                                                       | 650               | 13.8                        | 970                  | 47.9             | 3,350                | 47.1                |
|                            |                                                       | 750               | 13.0                        | 910                  | 34.0             | 2,380                | 52.2                |

TABLE I

| Temperature,<br>°C. | % Linear Expansion<br>$\frac{\Delta L}{L_{20^\circ\text{C.}}} \times 100$ |
|---------------------|---------------------------------------------------------------------------|
| 200                 | 0.26                                                                      |
| 400                 | 0.56                                                                      |
| 600                 | 0.92                                                                      |
| 800                 | 1.31                                                                      |
| 1000                | 1.78                                                                      |
| 1200                | 2.4                                                                       |
| 1400                | 2.78                                                                      |

These results, when plotted on a temperature-versus-percent linear expansion curve, reveal a smooth linear expansion from room temperature to 1,400° C., indicating no phase transformation occurring over the entire range of temperature, 0° to 1,400° C. An X-ray diffraction pattern taken from the specimen indicated that only the face-centered cubic austenitic phase was present.

## Precipitation Hardening

As previously mentioned, the maximum high-temperature strength of the alloy system within the scope of this invention can be developed if a suitable heat treatment is applied to the alloy in order to induce precipitation of a molybdenum-containing phase. This takes place in a two-step operation in which the first step consists of a solid solutioning heat treatment or homogenization at a temperature in the range 1,000° to 1,315° C. followed by a precipitation-inducing treatment and preferably at a temperature above the intended service design temperature. The solutioning step can be approached, in effect, by the use of a finish rolling temperature. The high-temperature solutioning heat treatment should be one which effects reasonably complete solutioning without causing excessive grain growth as determined by metallographic observation. The exact temperature or range of preferred temperature to achieve this effect for a given alloy is a function of the particular alloy composition and can be empirically determined by metallographic observation and hardness measurements. For an alloy containing 20 nickel, 5 percent chromium, and 10 percent molybdenum, a solutioning temperature of about 1,205° C. has been found to be satisfactory. The solutioned alloys are then aged at a temperature which will produce maximum and sustained hardness. Hardness ( $R_c$ ) curves for the Fe-20Ni-5Cr-10Mo alloy composition are presented in FIG. 1, which indicates the thermal treatment

### Short Term Tensile Properties

The purpose of this example is to demonstrate and compare the effects of a solution and aging heat treatment with the same alloy in the as-rolled and aged condition to determine the effect of the two processing methods on tensile strength and ductility. The results are summarized in Table II. For comparison purposes, tensile properties of a 316 stainless steel are included as representative of an alloy known to be useful over the same range of temperature.

It will be noted that the solution and age-hardening treatment have apparently resulted in an increase in ductility accompanied by slight decreases in yield strength and tensile strength at all temperatures from room temperature to 750°C. However, from an overall standpoint, the alloy demonstrates, with or without a precipitation heat treatment, a useful combination of tensile strength and ductility and higher tensile strength than the comparison 316 stainless steel.

## Creep

This example is intended to illustrate the effect of prior processing heat treatment history on the creep rupture properties of the Fe-20Ni-5Cr-10Mo alloy. In particular, it is designed to illustrate the effect of solutioning and precipitation-hardening on the creep properties of the alloy.

Sheet stock of the alloy were finish-rolled to 0.076 centimeter at two different temperatures, 750° and 982° C. Prior to the finish-rolling operation, one portion of sheet stock was aged at 750° C. for 20 hours while a second portion was solutioned at 1,200° C. for 1 hour, water quenched to room temperature, and then aged with 750° C. Both portions were finish-rolled at either 760° or 982° C. and the results are summarized in Table III below.

TABLE III.—EFFECT OF PROCESSING TEMPERATURE, HEAT TREATMENT, AND HEAT SIZE ON THE STRESS RUPTURE PROPERTIES<sup>a</sup> OF THE Fe-20Ni-5Cr-10Mo ALLOY

| Finish rolling temp., °C.                               | Heat treatment                                                          | Initial extension,<br>percent | Linear <sup>b</sup> creep rate,<br>in./in./hr. | Rupture life, hr. | Rupture elong., percent |
|---------------------------------------------------------|-------------------------------------------------------------------------|-------------------------------|------------------------------------------------|-------------------|-------------------------|
| At a Test Load of 1,960 kg./cm. <sup>2</sup> at 650° C. |                                                                         |                               |                                                |                   |                         |
| Sheet No.:                                              |                                                                         |                               |                                                |                   |                         |
| 1.....                                                  | 760 750° C.-20 hours.....                                               | 1.10                          | 2.4×10 <sup>-2</sup>                           | 11.6              | 43.9                    |
| 2.....                                                  | 760 .....do.....                                                        | 0.80                          | 4×10 <sup>-3</sup>                             | 35.2              | 41.4                    |
| 3.....                                                  | 982 .....do.....                                                        | 1.00                          | 2.6×10 <sup>-3</sup>                           | 66.8              | 37.5                    |
| 4.....                                                  | 982 .....do.....                                                        | 1.08                          | 3×10 <sup>-3</sup>                             | 68.2              | 38.1                    |
| 5.....                                                  | 982 .....do.....                                                        | 1.09                          | 2.5×10 <sup>-3</sup>                           | 73.3              | 28.0                    |
| 6.....                                                  | 760 1,200° C.-1 hours—<br>WQ <sup>c</sup> plus 750° C.-20<br>hours..... | 0.98                          | 1.1×10 <sup>-4</sup>                           | T>359.5           | T>3.6                   |
| 7.....                                                  | 760 .....do <sup>c</sup> .....                                          | 1.10                          | 5.8×10 <sup>-4</sup>                           | 238.3             | 21.5                    |
| 8.....                                                  | 982 .....do <sup>c</sup> .....                                          | 0.98                          | 6.5×10 <sup>-5</sup>                           | T>476             | T>3.4                   |
| 9.....                                                  | 982 .....do <sup>c</sup> .....                                          | 1.10                          | 5.3×10 <sup>-4</sup>                           | 288.2             | 21.1                    |
| 10.....                                                 | 982 .....do <sup>c</sup> .....                                          | 1.08                          | 3.6×10 <sup>-4</sup>                           | 463.6             | 24.7                    |
| 316SS.....                                              | Annealed at 1,120° C.....                                               | 4.05                          | 1.5×10 <sup>-3</sup>                           | 148.2             | 43.3                    |
| At a Test Load of 1,050 kg./cm. <sup>2</sup> at 750° C. |                                                                         |                               |                                                |                   |                         |
| 11.....                                                 | 760 750° C. 20 hours.....                                               | 0.55                          | 5.9×10 <sup>-2</sup>                           | 5.5               | 57.2                    |
| 12.....                                                 | 760 1,200° C.-1 hour-WQ <sup>c</sup><br>plus 750° C.-20<br>hours.....   | 0.83                          | 1.3×10 <sup>-5</sup>                           | T 596             | T1.7                    |
| 13.....                                                 | 982 .....do <sup>c</sup> .....                                          | 0.70                          | 2.7×10 <sup>-1</sup>                           | 295.1             | 16.4                    |
| 316SS.....                                              | Annealed at 1,120° C.....                                               | 0.54                          | 3.2×10 <sup>-3</sup>                           | 87.4              | 39.5                    |

T. No failure—test terminated.

a. Specimens were 0.076 cm. thick with a 0.63-cm.-wide reduced section and a 2.54-cm. gage length. The major axis of each specimen parallels the rolling direction. All tests on developmental alloys conducted in argon.

b. Extension based on dial gage reading of total train elongation and is approximate. Values for Type 316 stainless steel were read directly from gage section.

c. WQ = water quench.

The results show the dramatic improvement in rupture life obtained with a solid solution-precipitation heat treatment over the same alloy in the as-rolled-and-aged condition without the solutioning-precipitation heat treatment. A comparison of the rupture life of the solutioned and precipitation-heat-treated alloy with a 316 stainless steel shows similar significant improvements.

Creep rupture studies with lower amounts of molybdenum that we conducted showed that the same increased improvements cannot be obtained at molybdenum concentrations lower than about 5 percent.

Sheet specimens of the various heat-treated Fe-20Ni-5Cr-10Mo alloys were examined by electron microscopy techniques. Micrographs revealed coarse  $\mu$ -phase ( $Fe_7Mo_6$ ) particles present in the as-rolled condition at 982° C. which appeared to coalesce and dissolved when solutioned at 1,205° C. for 1 hour. A 1,315° C. solutioning dissolves essentially all particles but causes considerable grain growth. Aging each of the solutioned microstructures at 750° C. allows the  $Fe_7Mo_6$  to precipitate as crystallographically oriented platelets. The development of the  $\mu$ -phase platelets is believed to be primarily responsible for the higher creep rupture strength. The improvement in creep of the Fe-20Ni-5Cr-10Mo alloy can be illustrated in a somewhat different way by reference to FIG. 2, which is a Larson-Miller parametric representation of the Fe-20Ni-5Cr-10Mo alloy compared with a 316 stainless steel. In the equation, on the abscissa, T is temperature in °F., t is time in hours, and P is the parameter number—a dimension less constant. The curve clearly shows the strength advantage of the Fe-20Ni-5Cr-10Mo alloy over a considerable parametric range.

In recapitulation, it has been shown that a selected class of iron-base alloys containing a specifically defined range of concentration of chromium, nickel, and molybdenum subjected to a solutioning and precipitation-inducing heat treatment operation provides an alloy system which is completely

25 austenitic throughout the range of temperature from 0° to 1,400° C. In addition, this class of alloys has significant short- and long-term strength as well as ductility for use at service temperatures up to as high as 750° C. in nonoxidizing atmospheres.

30 For the sake of clarity, the concentration of the claimed alloy of this invention is given below in terms of weight percent as well as atom percent.

As an Fe-Ni-Cr-Mo alloy, the invention consists essentially of

|    | in atom percent | in weight percent |
|----|-----------------|-------------------|
| Fe | 50-71           | 46.29-68.56       |
| Ni | 20-30           | 20.30-29.19       |
| Cr | 5-10            | 4.50-8.62         |
| Mo | 4-10            | 6.64-15.90        |

As an Fe-Ni-Cr-W alloy, the invention consists essentially of

|    | in atom percent | in weight percent |
|----|-----------------|-------------------|
| Fe | 50-71           | 40.39-64.64       |
| Ni | 20-30           | 19.14-25.48       |
| Cr | 5-10            | 4.24-7.52         |
| W  | 4-10            | 11.98-26.61       |

What is claimed is:

1. An iron-base alloy characterized in that (a) it consists of an iron-nickel-chromium matrix which maintains substantially complete austenitic stability at temperatures from 0° to 1,400° C.; (b) it is susceptible to treatment to effect a precipitation-hardening resulting in a molybdenum-containing precipitated phase; (c) said alloy consisting essentially of, in weight percent, an iron-base alloy containing 20.30 to 29.19 percent nickel, 4.50 to 8.62 percent chromium, 6.64 to 15.90 percent molybdenum, and 46.29 to 68.56 percent iron.

2. An iron-base alloy characterized in that (a) it consists of an iron-nickel-chromium matrix which maintains substantially complete austenitic stability at temperatures from 0° to 1,400° C.; (b) it is susceptible to treatment to effect a precipitation-hardening resulting in a tungsten-containing precipitated phase; (c) said alloy consisting of, in weight percent, 19.14 to 25.48 percent nickel, 4.24 to 7.52 percent chromium, 11.98 to 26.61 percent tungsten, and 40.39 to 64.64 percent iron.

3. The alloy of claim 1 which consists essentially of, in weight percent, 19 to 20 percent nickel, 4 to 5 percent chromium, 15 to 16 percent molybdenum, and the balance iron.

\* \* \* \* \*